

## UNITED STATES PATENT OFFICE

CLARENCE I. ROBINSON, OF WEST NEW BRIGHTON, NEW YORK, ASSIGNOR TO  
STANDARD OIL DEVELOPMENT COMPANY, A CORPORATION OF DELAWARE

## HYDROCARBON OIL OF GOOD NONSMOKE RATING

No Drawing.

Application filed November 10, 1922. Serial No. 599,967.

My invention relates to the art of making hydrocarbon products, and will be fully understood from the following description.

For a long time illuminating oil prepared from Pennsylvania petroleum has stood as the superlative quality obtainable, being far superior to oils available from other petroleums. However not only is it merely a question of time when oil of this grade will be exhausted, but even at present with this oil, it is not possible to attain some particular results which have been desired in certain special signal usages.

In proceeding in accordance with my invention, one of the steps involved is a cracking or pyrolytic decomposition of the starting material employed, and the final results for the process are thus all the more surprising as it would be expected that a product derived from a cracking operation would be lacking in the non-smoking properties requisite in an illuminating oil.

As starting material I employ the paraffins which are normally solid when separated from the oils containing them. Ordinarily this separation is accomplished for example by chilling the oil or paraffin distillate, filter-pressing to segregate the paraffin and then maintaining the paraffin at a temperature short of its melting point but high enough to permit contained oil to ooze or sweat out. The paraffin may however be obtained in any other way desired. Complete purification is not necessary but may be resorted to if desired. In my experience a crude scale wax from mixed base crude petroleum and rating at around 98% crystalline paraffin, is a highly advantageous material. The paraffin in solid or melted state as most convenient, is charged into a still and subjected to cracking or pyrolytic decomposition at suitable temperatures, for example 675° to 750° F. being a good practical range, and pressure may or may not be employed, but if used would in general preferably not exceed 60 lbs. per square inch, as with increase of pressure and higher temperatures the yield runs more to light ends.

The overhead distillate obtained is separated into naphtha and refined oil; and the

products may be finished up in any desired way, advantageously for example, the distillate is first treated with 66° Bé. sulfuric acid, about 5 lbs. to the barrel of distillate, and is then distilled to remove the naphtha and the distillation is continued with fire and steam until the refined oil is off, or if desired the initial product may be first steam-stilled to remove naphtha and the residual oil then be treated with about 5 lbs. of acid per barrel and then be redistilled with fire and steam for finished refined oil. After the acid in either case a further treatment with caustic soda solution, with or without a final clay filtration, may be applied.

The naphtha obtained is a excellent gasoline and is characterized by an exceptionally high Baumé gravity (low specific gravity), showing for the Navy specification boiling range between 140° F. initial and 437° F. final, a gravity of 64°-66° Bé. as contrasted with the following recognized gasolines:

|                                               | Boiling range | Gravity   | 75 |
|-----------------------------------------------|---------------|-----------|----|
| From Pennsylvania oil.....                    | 140°-437° F.  | 62.0° Bé. |    |
| From Mid-Continent oil.....                   | 140°-437° F.  | 59.5° Bé. |    |
| From cracking gas oil from Mid-Continent..... | 140°-437° F.  | 58.5° Bé. |    |

The refined oil obtained is a very superior burning oil having a remarkably high Baumé gravity for the distillation range, which may be about 300-575° F. For example, for a distillation range of 350° F. to 560° F. it may have a gravity of over 50° Bé. It has a phenomenally high rating on the non-smoke-tendency test, viz. a rating of 125 to 185. The test here referred to is based upon Pennsylvania kerosene as a standard, a testing lamp having a flat wick and no chimney being used and the wick being turned as high as possible just short of smoking, the candle power is read on the photometer. This candle power reading on Pennsylvania kerosene is taken as 100 and the readings on other oils are rated proportional thereon. Another feature of this refined oil is the low sulfur content, this not

exceeding 0.025 and generally running as low as 0.012.

Comparative typical showing with various recognized kerosenes is as follows:

|                                  | Gravity | Acid absorption | Non-smoke rating |
|----------------------------------|---------|-----------------|------------------|
| Refined oil from present process | 50°-54° | 4-10%           | 175-185          |
| Pennsylvania kerosene            | 46°-49° | 3%              | 100              |
| Mid-Continent kerosene           | 42°-45° | 7%              | 40-60            |
| Pressure-Still kerosene          | 40°-43° | 12%             | 25-35            |

A sample of a refined oil made by the present process showed the following complete inspection:

|    | Gravity   | Color | Viscosity | Sulfur | Chill O. K. | Acid absorption | Non-smoke rating |
|----|-----------|-------|-----------|--------|-------------|-----------------|------------------|
| 20 | 51.6° Bé. | 21    | 370       | .012   | @ 0° F.     | 10%             | 185              |

#### Distillation:—

Initial 370° F.

25 15.25% off at 400° F.  
69.25% off at 450° F.  
92.75% off at 500° F.  
99.00% off at 554° F.

30 The general characteristics of the refined oil are a lower specific gravity for any given boiling point, and a higher viscosity and a higher non-smoke rating than that of products of the same boiling point from petroleum.

35 Inspections made on samples from various runs with and without pressure show the practical characteristics of the product as gravity 49.5°-55° Bé., viscosity 330 to 460 at 60° F., on the Saybolt thermo-viscometer, sulfur not in excess of 0.025, acid absorption (using 66° Bé. sulfuric acid) 4-10% and non-smoke rating 125-185.

40 Not only is a high candle-power for a petroleum product realized with this oil as indicated above under the non-smoke tendency test, it yielding 75 to 85% more candle power than Pennsylvania kerosene on a given wick without smoking, but the oil burns without formation of wick-crusts. 45 In consequence it makes possible the operation of special signal lamps or other lamps burning for three or four weeks or more without any attention.

50 It will be understood that the crude scale paraffin as above referred to is the most advantageous starting material but even with a paraffin less fully freed from oil, the advantages of my invention are attained in proportion, the product being of course proportionally poorer as the percentage of contaminating oil is increased, and with material in which the paraffin is mingled with substantial portions of oil, it is advisable that the oil content should be within

such limits that the material will not be liquid at temperatures lower than 90° F.

Besides the paraffin from petroleum, paraffin from other sources, such as from shale oils, and low temperature coal retorting, may be used.

70 While in describing my invention I have referred to certain specific details, it will be understood that this is by way of illustration and explanation, and is not limitative. The invention is to be regarded as limited only as defined in the following claims, in which it is my intention to claim all inherent novelty as broadly as the prior art permits.

#### What I claim is:

1. A hydrocarbon product characterized by a distillation range between 350° and 560° F., a gravity of 50° to 54° Bé., a viscosity between 330 and 460 at 60° F. on the Saybolt thermo-viscometer, and an acid absorption of 4-10% and a non-smoke rating of 175-185.

2. A hydrocarbon product having a distillation range between 300° and 575° F., a gravity of 49.5°-55° Bé. and a non-smoke rating in excess of 125.

3. A hydrocarbon product having a distillation range between 300° and 575° F., and a non-smoke rating in excess of 125.

95 CLARENCE I. ROBINSON.

80

85

90

95

100

105

110

115

120

125

130